

## UNITED STATES PATENT OFFICE.

JOHN L. COX, OF PHILADELPHIA, PENNSYLVANIA.

## STEEL ALLOY.

No Drawing.

Application filed February 12, 1927. Serial No. 167,873.

My invention relates to a steel alloy and more especially to a steel alloy adapted for use under conditions of relatively high temperature. The alloy in accordance with my 5 invention is especially adaptable for use in the construction of valves and for the construction of which a steel alloy containing chromium and tungsten has heretofore been used.

10 Valve steels containing chromium and tungsten are open to a serious objection in that at high temperatures tungsten steel scales very badly, so that after a short run at a temperature of, say, as high as 1600° F. 15 scale will fall from the surface of a valve in sheets, interfering with the proper seating of the valve and destroying the seating surface.

In an effort to prevent the scaling of 20 tungsten steel articles, such as valves, the articles have been subjected to the so-called calorizing process which consists in impregnating the surface of the article with aluminum, which on heating oxidizes and 25 protects the material beneath. Calorizing is, however, not a satisfactory remedy, since the surface only of the article is protected and where the article is a valve only a limited amount of grinding may be performed 30 before the effect of the calorizing is lost.

Now, it is the object of my invention to provide a steel alloy including chromium and tungsten, which will not scale under 35 conditions of high temperature and which will lend itself especially to use as a valve steel.

In accordance with my invention I form 40 a steel alloy containing chromium and tungsten, in such proportions as are usually met with in steel making practice, and in addition aluminum, the aluminum being incorporated in the composition of the original metal and being uniform in amount throughout the steel. The aluminum may 45 be present in amount ranging from 1% to 6% depending upon the amount of chromium and tungsten present.

The steel alloy embodying my invention

may contain the following ingredients within the ranges specified:—

|                                 | Per cent. |    |
|---------------------------------|-----------|----|
| Carbon, from                    | 0.5- 1.50 |    |
| Chromium, from                  | 4.0-20.0  |    |
| Tungsten, from                  | 6.0-18.0  |    |
| Aluminum, from                  | 1.0- 6.0  | 55 |
| The remainder principally iron. |           |    |

A typical composition embodying my invention is the following:—

|                                 | Per cent. |    |
|---------------------------------|-----------|----|
| Carbon, about                   | 0.75      | 60 |
| Chromium, about                 | 8.0       |    |
| Tungsten, about                 | 14.5      |    |
| Aluminum, about                 | 3.0       |    |
| The remainder principally iron. |           |    |

Another typical composition embodying my invention is the following:—

|                 | Per cent. |    |
|-----------------|-----------|----|
| Carbon, about   | 0.9       |    |
| Chromium, about | 14.5      |    |
| Tungsten, about | 6.25      | 70 |
| Aluminum, about | 1.85      |    |

In general, the percentage of aluminum should increase as the percentage of tungsten increases, but not necessarily in the same proportion; that is, an alloy relatively high in tungsten should contain more aluminum than an alloy relatively low in tungsten.

It will be understood that other alloys may be included in the composition of the steel alloy without departing from my invention, it being noted, for example, that silicon may be added within the ranges usually encountered in steel making practice, which varies from .05 to 1.75 per cent.

In the composition according to my invention molybdenum may be substituted for tungsten in whole or in part. However, when molybdenum is substituted for tungsten, whether in whole or in part, it should be substituted for tungsten in the proportion of from  $\frac{1}{3}$ - $\frac{1}{2}$  of the tungsten, and where, in the claims, proportions of tungsten are specified, molybdenum, in the lesser proportion stated, is to be considered an equivalent of tungsten.

In the steel alloy according to my invention, the aluminum, being more oxidizable than the iron, chromium or tungsten, is first attacked by oxygen and forms a protective 5 coating, which is firmly adherent and beneath which the oxidation of the other metals proceeds but slowly.

The aluminum, since it is incorporated in the composition of the original metal, is 10 uniformly distributed in amount throughout the steel and the protective coating formed is continuously renewed as the surface wears. When the steel is used for the production of a valve, the protective coating 15 is continuously renewed as the valve wears and the valve may be ground without fear of subsequent scaling, since the aluminum distributed through the mass of the valve will oxidize and renew the protective 20 coating removed by wear or grinding.

In the steel alloy in accordance with my invention the advantages of hardness, etc., inherent in tungsten steels are retained and the scaling is entirely suppressed. Under 25 conditions of high temperature the steel, with certain composition within the ranges mentioned by me, will suffer only such discoloration as would occur in the tempering of a polished hardened steel article, while 30 with other compositions the steel may become coated with a dark oxide, which is usually firmly adherent and will not flake off.

Having now fully described my invention, 35 what I claim and desire to protect by Letters Patent is:—

1. A forgeable steel alloy containing carbon .35-1.5%, chromium 4-20%, tungsten 6-18% and aluminum 1-6%, the remainder 40 and dominating proportion of the composition being principally iron, the proportion of tungsten being not less than one-fourth the proportion of chromium and the proportion of aluminum being not less than one-sixth 45 the proportion of tungsten.

2. As a new article of manufacture, a forged valve composed of a steel alloy comprising carbon .35-1.5%, chromium 4-20%, tungsten 6-18%, and aluminum 1-6%, the 50 proportion of tungsten being not less than one-fourth the proportion of chromium and the proportion of aluminum being not less

than one-sixth the proportion of tungsten, the remainder and dominating proportion of the composition being principally iron, said valve being characterized, at high temperatures, by being substantially non-scaling and comparatively hard. 55

3. A steel alloy containing carbon .35 to 1.5 per cent, chromium 4 to less than 20 per cent, tungsten 6 to 18 per cent, aluminum 1 to 6 per cent and silicon not over 1.75 per cent, the remainder and dominating proportion of the composition being principally iron, the proportion of aluminum being not 65 less than one-sixth the proportion of tungsten.

4. As a new article of manufacture, a forged valve composed of a steel alloy comprising carbon .35 to 1.5 per cent, chromium 4 to less than 20 per cent, tungsten 6 to 18 per cent, aluminum 1 to 6 per cent and silicon not over 1.75 per cent, the remainder and dominating proportion of the composition being principally iron, said valve being 70 characterized, at high temperatures, by being substantially non-scaling and comparatively hard. 75

5. A steel alloy containing carbon .35 to 1.5 per cent, chromium 4 to less than 10 per cent, tungsten 6 to 18 per cent, aluminum 1 to 6 per cent and silicon not over 1.75 per cent, the remainder and dominating proportion of the composition being principally iron, the proportion of aluminum being not 85 less than one-sixth the proportion of tungsten.

6. As a new article of manufacture, a forged valve composed of a steel alloy comprising carbon .35 to 1.5 per cent, chromium 4 to less than 10 per cent, tungsten 6 to 18 per cent, aluminum one to 6 per cent, and silicon not over 1.75 per cent, the remainder and dominating proportion of the composition being principally iron, said valve being characterized, at high temperatures, by 95 being substantially non-scaling and comparatively hard.

In testimony of which invention, I have hereunto set my hand, at Philadelphia, 100 Pennsylvania, on this twelfth day of February, 1927.

JOHN L. COX.